

Oct. 11, 1938.

M. O. SCHUR

2,132,863

MULTIPLE IMPREGNATION OF COMPRESSIBLE FIBROUS WEBS

Filed Aug. 4, 1936



Invention  
Milton O. Schur  
by Wright, Brown, Quincy & May  
Attest

## UNITED STATES PATENT OFFICE

2,132,863

## MULTIPLE IMPREGNATION OF COMPRESSIBLE FIBROUS WEBS

Milton O. Schur, Berlin, N. H., assignor to Brown Company, Berlin, N. H., a corporation of Maine

Application August 4, 1936, Serial No. 94,156

5 Claims. (Cl. 91—68)

This invention relates to multiple impregnation of a compressible fibrous web, that is, to the impregnation of such a web with different impregnants or with different amounts or concentrations of the same impregnant at different portions of the depth or body of the web.

It is sometimes the practice to produce impregnated fibrous webs or sheets of the foregoing character by superimposing and bonding together two or more plies each impregnated with the desired material or to the desired impregnant concentration. Not only is the impregnation of individual plies and their bonding or plying unduly expensive in some cases, but it is sometimes difficult to work with thin plies, for instance, thin paper plies such as are to be impregnated with aqueous binder compositions and to serve as surface layers in the finished plied product.

20 In accordance with the present invention, I produce from a compressible single fibrous web an impregnated sheet whose surface portion is impregnated with a different material or concentration of the same material than the interior portion or layer of the sheet. A practice embodying the invention hereof may, for example, involve passing a compressible fibrous web or foundation through a bath of impregnating liquid binder, then subjecting the wet impregnated web to light mechanical squeezing, as by passage through squeeze rolls, and then passing the squeezed wet web over a "kiss" or applicator roll rotating partially submerged in another or secondary liquid binder which it is desired to incorporate into the surface portion of the web. Because the wet impregnated web has been slightly squeezed, it is capable of imbibing the secondary liquid binder and does so immediately upon being brought into contact 30 with the film of liquid binder on the kiss roll. The infusion of the secondary liquid binder into the web preferably takes place promptly after the squeezing of the web so as to avoid undesirable setting of the first liquid binder in the surface portion of the web as the squeezed web tends to recover its original thickness. The application of secondary liquid binder to the web may, however, be delayed slightly after the squeezing of the web in those instances when the primary liquid binder does not tend to set or congeal rapidly; and, in such latter case, the amount of secondary binder that can be added to the web is greater than when such binder is infused into the web immediately after its squeezing, that is, before the web has had op-

portunity of recovering part or much of its original thickness.

In the accompanying drawing,—

Figure 1 illustrates diagrammatically and conventionally the practice of a method embodying the present invention.

Figures 2, 3, and 4, represent sections through typical multiply-impregnated products such as might be produced by such method.

As appears in Figure 1, a web or sheet S of 10 compressible fibrous material may be progressively unwound from a roll R and passed through a bath B of primary liquid binder such as may be desired in the main body portion of the web. As the impregnated web comes from the bath, 15 it may enter the nip of a pair of squeeze rolls C whose peripheries clear each other by a gap slightly less, for instance, about .003 to .006 inch, than that of the thickness of the original or dry web, which may have an original 20 thickness of, say, about 0.030 to 0.060 inch and which may swell or expand somewhat as a result of impregnation with the primary liquid binder. The squeezed web may then be passed into contact with a film of secondary liquid 25 binder on the periphery of a kiss roll K rotating partially submerged in a bath of the secondary liquid binder L, whereupon the multiply-impregnated web may undergo such further treatment as is necessary to cause the two binder 30 compositions therein to set or congeal.

By the foregoing method, it is possible, for instance, to impregnate the body of a felted fibrous web throughout with rubber latex as the primary impregnant, then to drive or dislodge 35 the rubber latex to a greater or lesser degree from the surface portions of the web by squeeze rolls, and then to replace the dislodged rubber latex with aqueous albuminous binder, for instance, glue solution. The resulting multiply-40 impregnated web may then be dried, as by passage through a hot-air drying chamber or over steam-heated drum driers. The resulting product thus impregnated mainly with rubber but comprising a surface portion impregnated with 45 glue, which is shown in Figure 2, is of value as artificial leather for shoe innersoles and other uses wherein it is desired that the artificial leather surface be substantially devoid of rubbery feel.

Rather than incorporating aqueous albuminous binder as a secondary binder into the surface portion of the wet impregnated web after its squeezing, I may employ glycerine as a secondary impregnant, for instance, when a fin- 50 55

ished product having a comparatively porous surface portion is desired, that is, a surface portion poor in rubber relative to the main body of the finished sheet, as depicted in Figure 3. It 5 might be noted that the incorporation of glycerine into the surface portion of the wet impregnated web after its squeezing tends to eliminate the otherwise prevalent tendency for the rubber latex to diffuse back to the web surface, since 10 glycerine occupies to a large extent the surface pores of the web and diffusion or migration of the rubber particles through the comparatively viscous glycerine or glycerine solution is so greatly retarded that the rubber particles are set 15 before much diffusion has occurred.

In some instances, it may be desirable to produce an impregnated fibrous sheet of comparatively low rubber content in its main body portion but rich in rubber in its surface layer or portion, as when the surface is to be finished with nitrocellulose or other lacquer or liquid finish and loss or absorption of the finish in the body of the sheet is to be avoided. In such cases, the main body of the fibrous web may be impregnated 20 as a whole with a relatively dilute latex composition and then, after the impregnated web has been squeezed, its surface portion may be made to imbibe a comparatively concentrated latex composition, namely, one which upon drying 25 of the multiply-impregnated web deposits sufficient rubber and other solids in the surface layer or portion to clog to a desirable degree the pores and interstices in such layer against material influx of such liquid finish as may be subsequently applied thereto.

In producing the various multiply-impregnated products hereinbefore described for purpose of illustration, it is possible to work successfully with the compressible absorptive fibrous bases or webs 40 fabricated from cellulose pulp, for instance, wood pulp, rag pulp, and other fiber furnishes on paper-making machines. Of course, carded webs or felts fabricated from cotton, wool, and other textile fibers, compressible woven cloths, and other 45 compressible fibrous fabrics might serve as the foundations or bases being impregnated.

I claim:

1. A method which comprises impregnating substantially throughout its body with an aqueous 50 impregnating composition a cellulose fiber web tending to swell upon impregnation with such composition but being compressible to less than its original thickness, compressing the resulting impregnated and swollen web to less than the 55 original web thickness and thereby dislodging aqueous impregnating composition from its surface portion, and infusing secondary liquid impregnant substantially only into said surface portion while the web is still recovering from its compressed condition and it is still wet with said aqueous impregnating composition.

2. A method which comprises progressively passing through a bath of aqueous impregnating composition a felted cellulose fiber sheet tending to swell upon immersion in and impregnation with said composition but being compressible to less than its original thickness, progressively compressing the resulting swollen and impregnated sheet, as it emerges from said bath, to less than the original sheet thickness and thereby dislodging aqueous impregnating composition 10 from its surface portion, and progressively applying secondary liquid impregnant as a coating to the surface of said compressed sheet while it is still recovering from its compressed condition and it is still wet with said aqueous impregnating composition. 15

3. A method which comprises impregnating substantially throughout its body with rubber latex composition a cellulose fiber web tending to swell upon impregnation with such composition but being compressible to less than its original thickness, compressing the resulting impregnated and swollen web to less than the original web thickness and thereby dislodging rubber latex composition from its surface portion, and infusing 20 a secondary liquid impregnant substantially only into said surface portion while the web is still recovering from its compressed condition and it is still wet with said rubber latex composition. 25

4. A method which comprises progressively 30 passing through a bath of rubber latex composition a felted cellulose fiber sheet tending to swell upon immersion in and impregnation with said composition but being compressible to less than its original thickness, progressively compressing 35 the resulting swollen and impregnated sheet, as it emerges from said bath, to less than the original sheet thickness and thereby dislodging rubber latex composition from its surface portion, and progressively applying aqueous albuminous binder composition as a coating to the surface of said compressed sheet while it is still recovering from its compressed condition and it is still wet with said rubber latex composition. 40

5. A method which comprises progressively 45 passing through a bath of relatively dilute rubber latex composition a felted cellulose fiber sheet tending to swell upon immersion in and impregnation with said composition but being compressible to less than its original thickness, progressively 50 squeezing the resulting swollen and impregnated sheet, as it emerges from said bath, to less than the original sheet thickness and thereby dislodging rubber latex composition from its surface portion, and progressively applying a relatively concentrated rubber latex composition as a coating to the surface of said compressed sheet while it is still recovering from its compressed condition and it is still wet with said relatively dilute rubber latex composition. 55

MILTON O. SCHUR.

60